

## UNITED STATES PATENT OFFICE

2,153,927

CYANINE DYES AND A PROCESS FOR  
PREPARING THEMJohn David Kendall, Ilford, England, assignor to  
Ilford Limited, Ilford, England, a British companyNo Drawing. Application December 21, 1934,  
Serial No. 758,647. In Great Britain December  
23, 1933

11 Claims. (Cl. 260—240)

This invention consists in improvements in or relating to the production of compounds containing an ethylenic linkage, or a methine or a polymethine chain, and more particularly to compounds containing two polyvalent elements or groups of elements joined together by such a linkage or chain.

The methine chain consists of the group



in which X represents hydrogen or any other monovalent non-metallic element or grouping. 15 The polymethine chain contains a number of methine groups, an example being



20 Such a chain may be extended and one or more of the hydrogen atoms may be substituted as in the simple methine chain.

According to the present invention a process for the production of compounds containing an 25 ethylenic or a methine or polymethine chain comprises reacting a body containing the group:



(where R<sub>1</sub>, R<sub>2</sub> and R<sub>3</sub> may be hydrogen, alkyl, aryl or aralkyl groupings, or R<sub>1</sub> and R<sub>2</sub> may be part of an arylene residue as in indene) with a 35 quaternary salt of a heterocyclic nitrogen compound containing a thio ether or seleno ether grouping including aryl or aliphyl or araliphyl thioethers and selenoethers. The quaternary salt of the thio or seleno ether may be derived from an 40 alkyl thione or selenone by reacting with an alkyl salt, as is shown by the following general formula in which X represents the remainder of a heterocyclic radical, R is an alkyl radical and Y is an acid radical:



50 in each case the quaternary salt of the thio or seleno ether may be formed either before or simultaneously with the reaction with the cyclopentadiene compound.

Examples of compounds containing the groupings



are plain and substituted cyclopentadienes and indenes.

Examples of compounds containing reactive thioether, thione or like groupings which can be 10 condensed with the bodies of the type described are those having a reactive alkyl, aryl or aralkyl mercapto group in the  $\alpha$  or  $\gamma$  position such as quaternary salts of the following compounds which may be substituted or unsubstituted: 15 alkyl quinoline-2-thiones, alkyl mercaptothiazoles, alkyl mercapto oxazoles, alkyl mercapto pyridines alkyl mercapto diazoles, alkyl mercapto quinazolines, alkyl mercapto pyrimidines, alkyl mercapto phthalazines and alkyl mercapto indolenines (e. g. a 2-methylmercapto-3:3-dimethylindolenine).

These two types of compounds interact (in the manner shown in the following general equation) to form a new type of carbocyanine compound (of the general formula given in the following equation) in which the polymethine chain of the normal carbocyanine compound is replaced by the cyclopentadiene nucleus:



35 in the above general formulae R<sub>1</sub>, R<sub>2</sub> and R<sub>3</sub> may be hydrogen, alkyl, aryl or aralkyl groupings, or R<sub>1</sub> and R<sub>2</sub> may be part of an arylene radical, Y is an acid radical and X represents the remainder of a heterocyclic radical.

40 Many of the dyes produced in accordance with the invention influence the sensitivity of photographic sensitive emulsions to which they are added or which may be bathed in their solutions, and some may be employed for dyeing materials such as textiles.

Several specific examples are given below in order to illustrate the process according to the invention.

5 CYCLOPENTADIENE CONDENSATION

EXAMPLE I

10 *2,2'-dimethyl-7,7'-di-methenyl-thiocarbocyanine bromide* having the structural formula



15 5 gm. of methylmercapto benzthiazole and 5.2 gm. of methyl-p-toluene sulphonate were heated together for 4 hours at 130°-140° C. 6 cc. of cyclopentadiene and 20 cc. of pyridine were then added and the mixture was refluxed for 3/4 hour. It was then poured into an aqueous solution of potassium bromide and allowed to stand when a precipitate was formed. This was filtered off and recrystallised from hot spirit to give yellow crystals melting at 252° C., with decomposition.

20 This dye so produced is a sensitiser for silver chloride emulsions and sensitises over a band from  $\lambda$  4600-5700 Å. with a maximum at  $\lambda$  4950 Å.

25

EXAMPLE II

30 *2,2'-diethyl-7,7'-di-methenyl-thiocarbocyanine bromide*

35 This compound was prepared in a manner similar to that described in Example I but using ethyl-p-toluene sulphonate. The product was a dye in the form of yellow crystals, melting at 265° C. with decomposition. This dye is a sensitiser for silver chloride emulsion sensitising over a band from  $\lambda$  4600 to 6100 Å., with a maximum at  $\lambda$  4950 Å.

40 The corresponding iodide *2,2'-diethyl-7,7'-ethylene-thiocarbocyanine-iodide* was obtained, 45 in a similar manner with the substitution of potassium iodide solution for the potassium bromide solution as yellow crystals melting at 265° C.

45 This dye is a sensitiser for silver chloride and iodobromide emulsions and sensitises over a band 50 from  $\lambda$  4400-5300 Å., with a maximum at about  $\lambda$  5000 Å.

EXAMPLE III

55 *1,1'-dimethyl-9,9'-di-methenyl-2,2'-carbocyanine bromide*, having the structural formula



60 2.5 gm. of 1-methyl-quinoline-2-thione and 2.7 gm. of ethyl p-toluene sulphonate were heated together for four hours at 130°-140° C. 5 cc. of cyclopentadiene and 20 cc. of pyridine were then added and the mixture refluxed for one hour. The mixture was then poured into an aqueous solution of potassium bromide when a solid separated out which was filtered off and recrystallised from methyl alcohol to give red brown crystals melting at 268° C.

65 This dye is a sensitiser for silver iodobromide emulsions and extends the sensitivity to about  $\lambda$  6200 Å. with a maximum at about  $\lambda$  5700 Å.

EXAMPLE IV

70 *1,1'-diethyl-9,9'-di-methenyl-2,2'-carbocyanine bromide*

75 This compound was obtained, as green crystals melting at 268° C., from 1-ethyl quinoline-2-thione by a method similar to that described in Example III.

80 This dye is a sensitiser for silver iodobromide emulsions and extends the sensitivity to  $\lambda$  6200 Å. with a maximum at  $\lambda$  5800 Å.

EXAMPLE V

85 *2,2'-dimethyl-4,5,4',5'-tetraoxy-dimethenyl-7,7'-di-methenyl-thio-carbocyanine-p-toluene sulphonate* was obtained by a method similar to that of Example III from 1-methylmercapto-4,5-dioxymethylene benzthiazole, methyl-p-toluene sulphonate, and cyclopentadiene, as red needles 90 with a blue reflex, melting at 308° C.

95 The dye is a sensitiser for silver chloride and iodobromide emulsions sensitising over a band from about  $\lambda$  4400-5700 Å. with a maximum at about  $\lambda$  5200 Å.

EXAMPLE VI

100 *2,2'-diethyl-4,5,4',5'-tetraoxy-dimethenyl-7,7'-di-methenyl thiocarbocyanine-p-toluene sulphonate* was prepared by a method similar to that of Example III, using ethyl-p-toluene sulphonate, as brown yellow crystals melting at 295° C.

105 The dye is a sensitiser for silver chloride and iodobromide emulsions sensitising over a band from about  $\lambda$  4400 to 5700 Å. with a maximum at about  $\lambda$  5200 Å.

EXAMPLE VII

110 *2,2'-dimethyl-4,5,4',5'-tetramethoxy-7,7'-di-methenyl-thiocarbocyanine-p-toluene sulphonate* was obtained by a method similar to that of Example III, from 1-methyl-mercapto-4,5-dimethoxy-benzthiazole-ethyl-p-toluene sulphonate and cyclopentadiene, as orange yellow crystals 115 melting at 296° C.

120 The dye is a sensitiser for silver chloride and iodobromide emulsions sensitising over a band from about  $\lambda$  4000 to  $\lambda$  5900 Å. with an indeterminate maximum at about  $\lambda$  4800 Å.

EXAMPLE VIII

125 *2,2'-diethyl-4,5,4',5'-tetramethoxy-7,7'-di-methenyl-thiocarbocyanine-p-toluene sulphonate* was obtained by a method similar to that of Example III, from 1-methylmercapto-4,5-dimethoxy-benzthiazole-ethyl-p-toluene sulphonate and cyclopentadiene, as orange red crystals melting at 280° C.

130 The dye is a sensitiser for silver chloride and iodobromide emulsions and sensitises over a band from about  $\lambda$  4400 to 5700 Å. with an indeterminate maximum at about  $\lambda$  5100-5200 Å.

EXAMPLE IX

135 *A thiocarbocyanine from di-methylmercapto thio  $\beta,\beta'$  diazole and cyclo pentadiene*, having the structural formula



140

145

2.6 gm. of di-methylmercapto thio- $\beta,\beta'$ -diazole which has the structural formula:



and 5.6 gm. of methyl-p-toluene sulphonate were 10 heated together for four hours at 130-140° C. 8 cc. of cyclopentadiene and 20 cc. of pyridine were then added and the mixture refluxed for 1 hour after which it was poured into an aqueous solution of potassium iodide. On standing dark 15 green crystals separated out and were filtered off, washed and this precipitate was boiled with 180 cc. of spirit and filtered hot and the filtrate allowed to cool when yellow crystals melting at 224° C. were deposited. 20 The dye is a sensitiser for silver chloride emulsion and sensitises over a band from about  $\lambda$  4200-5000 Å. with a maximum at about  $\lambda$  4750 Å.

25 EXAMPLE X

A thiocarbocyanine iodide dyestuff was obtained by a method similar to that of Example IX from dimethylmercapto thio  $\beta,\beta'$  diazole, ethyl p-toluene sulphonate and cyclo pentadiene, 30 as small yellow needles melting at 202° C.

The dye is a sensitiser for silver chloride and 35 iodo bromide emulsions sensitising over a band from about  $\lambda$  4200-5100 Å. with a maximum at about  $\lambda$  4800 Å.

EXAMPLE XI

2,2'-dimethyl-3,4,3',4'-dibenz-7,7 - di - methyl-thio-carbocyanine-p-toluene sulphonate, was obtained by a method similar to that of Example 40 IX, from 2-methylmercapto  $\beta$  naphthathiazole-methyl-p-toluene sulphonate, and cyclo pentadiene, as orange red needles melting at 226° C. The dye is a sensitiser for silver iodobromide 45 emulsions and extends the sensitivity to about  $\lambda$  5700 Å. with a maximum at about  $\lambda$  5300 Å.

EXAMPLE XII

50 2,2'-dimethyl - 7,7' - dimethenyl - oxacarbocyanine bromide was prepared by a method similar to that of Example IX from 1-methylmercapto benzoxazole, methyl-p-toluene sulphonate and cyclo pentadiene as yellow crystals melting at 240° C.

55 INDENE CONDENSATIONS—CONDENSATION WITH THIONES

EXAMPLE XIII

60 1,1'-dimethyl 9,9'-phenylene 2,2'-carbocyanine-p-toluene sulphonate—5 gm. of indene 8 gm. of methyl-quinoline-2-thione and 9 gm. of ethyl-p-toluene sulphonate were heated together at 130-140° C. for four hours. 15 cc. of pyridine 65 were then added and the mixture refluxed for a quarter of an hour when the mixture became solid. The flask was washed out with some spirit and the crystals filtered off and washed with water and ether and recrystallised from methyl alcohol to give green needles, melting at 273° C.

The dye is a sensitiser for silver iodobromide emulsions and extends the sensitivity to about  $\lambda$  7000 Å. with a maximum at about  $\lambda$  6600 Å. and 70 a minimum at about  $\lambda$  5400 Å.

EXAMPLE XIV  
1,1'-diethyl-9,9'-o-phenylene-2,2'-carbocyanine bromide

3 gm. of 1-ethylquinoline-2-thione and 3.2 gm. of ethyl-p-toluene sulphonate were heated for four hours at 130-140° C. 3.8 gm. of indene and 2.5 cc. pyridine were then added and the mixture refluxed for an hour after which it was poured into an aqueous solution of potassium bromide. 10 Glistening bronze crystals were formed which were filtered off and recrystallised from dry spirit to give green crystals melting at 215° C.

CONDENSATIONS WITH METHYLMERCAP- 15 TO COMPOUNDS

EXAMPLE XV  
2,2'-dimethyl-7,7'-o-phenylene thiocarbocyanine iodide

2.5 gm. of indene, 8 gm. of 1-methylmercapto-benzthiazole and 8.5 gm. of methyl-p-toluene sulphonate were heated together at 130-140° C. for 4 hours. 20 cc. of pyridine were added and the mixture refluxed for 1 hour after which it was poured into an aqueous solution of potassium bromide. The solid which separated out was filtered off, washed with water, hot benzene and ether, and recrystallised from methyl alcohol, 25 to give red needles melting at 245° C. with decomposition. The dye is a sensitiser for silver iodobromide emulsions and extends the sensitivity to about  $\lambda$  5900 Å. with a maximum at about  $\lambda$  5700 Å.

EXAMPLE XVI

2,2'-diethyl-7,7'-o-phenylene - thio - carbocyanine-p-toluene sulphonate was obtained by a method similar to that of Example XV using water in place of the potassium bromide solution, as 40 scarlet needles. By pouring the reaction mixture into potassium iodide solution as before the corresponding iodide was obtained as red needles melting at 226-8° C.

Both these dyes are sensitisers for silver iodo- 45 bromide emulsions and extend the sensitivity to about  $\lambda$  6000 Å. with a maximum at about  $\lambda$  5600 Å.

EXAMPLE XVII

2,4,6,2',4',6'-hexamethyl-7,7'-o-phenylene - oxacarbocyanine-iodide was prepared by a method similar to that of Example XV, from indene, 1-methylmercapto - 4.5-dimethyl-benzoxazole and 55 methyl-p-toluene sulphonate, as yellow brown powder melting at over 300° C.

EXAMPLE XVIII

Dimethyl - o-phenylene-phthalazocarbocyanine 60 iodide having the structural formula



70 This salt was prepared by a method similar to that of Example XV from methyl mercapto-phthalazine, indene, and methyl-p-toluene sulphonate to give a purple dyestuff. The dye is a desensitiser for silver iodobromide emulsions.

## EXAMPLE XIX

A number of compounds were prepared from methyl-mercapto bodies and indene by the following general method:

5 The methyl mercapto body together with the alkyl-p-toluene sulphonate were heated for about four hours at 130-140° C. The indene was then added together with some pyridine and the mixture refluxed for half to one hour after which it was poured into water if the p-toluene sulphonate of the dye was required or into a solution of the appropriate alkali salt, such as potassium iodide, if a different dye salt was required. The precipitate was filtered off, washed and recrystallised from a suitable solvent usually spirit or methyl alcohol.

10 Examples of compounds prepared by this method are as follows:

15 *2,2'-dimethyl-7,7'-o-phenylene-oxacarbocyanine-iodide* was prepared from indene, 1-methyl-mercapto-benzoxazole, and methyl-p-toluene sulphonate to yield green crystals with a blue reflux, melting at 270° C. The dye is a sensitiser for silver chloride emulsions and sensitises over a band from about  $\lambda$  4200-5060 Å., with a maximum at  $\lambda$  4860 Å.

20 *2,2'-dimethyl-4,5,4',5'-tetraoxy dimethylene-7,7'-o-phenylene-thiocarbocyanine-p-toluene sulphonate* was prepared from 1-methylmercapto-4,5-dioxymethylene benzthiazole, indene, and methyl-p-toluene sulphonate, as pale pink needles melting at 244° C.

25 The dye is a sensitiser for silver chloride and iodobromide emulsions and extends the sensitivity to about  $\lambda$  6000 Å. with a maximum at about  $\lambda$  5700 Å.

30 *2,2'-diethyl-4,5,4',5'-tetraoxydimethylene-7,7'-o-phenylene-thiocarbocyanine-p-toluene sulphonate* was prepared from 1-methylmercapto-4,5-dioxymethylene benzthiazole, indene and ethyl-p-toluene sulphonate, as green needles melting at 295° C. The dye is a sensitiser for silver chloride and iodobromide emulsions and extends the sensitivity to  $\lambda$  6200 Å. with a maximum at  $\lambda$  5800 Å.

35 *2,2'-dimethyl-4,5,4',5'-tetra methoxy-7,7'-o-phenylene-thiocarbocyanine bromide* was prepared from 1-methyl-mercapto-4,5-dimethoxy benzthiazole, indene, and methyl-p-toluene sulphonate, as golden crystals melting at 260° C. The dye is a sensitiser for silver chloride and iodobromide emulsions and extends the sensitivity to about  $\lambda$  6100 Å. with a maximum at about  $\lambda$  5600 Å.

40 *2,2'-diethyl-4,5,4',5'-tetramethoxy-7,7'-o-phenylene-thiocarbocyanine bromide* was prepared from 1-methylmercapto-4,5-dimethoxy benzthiazole, indene, and ethyl-p-toluene sulphonate, as red needles melting at 258° C. The dye is a sensitiser for silver chloride and iodobromide emulsions and extends the sensitivity to about  $\lambda$  6300 Å. with a maximum at about  $\lambda$  5600 Å.

45 The bromide salt of a dyestuff was obtained from dimethyl-mercapto-thio- $\beta,\beta'$ -diazole, indene and methyl-p-toluene sulphonate, as red brown needles melting at 218°. The dye is a sensitiser for silver iodo bromide emulsions and extends the sensitivity to about  $\lambda$  5700 Å. with a maximum at about  $\lambda$  5400 Å.

50 The bromide salt of a dyestuff was obtained from dimethyl-mercapto-thio- $\beta,\beta'$ -diazole, indene, and ethyl-p-toluene sulphonate, as blue needles melting at 202° C. The dyestuff is a

5 sensitiser for silver chloride iodobromide emulsions and extends the sensitivity to about  $\lambda$  5600 Å. with a maximum at about  $\lambda$  5250 Å.

10 The bromide salt of a dyestuff was obtained from dimethyl-mercapto-thio- $\alpha,\beta'$ -diazole, indene, and methyl-p-toluene sulphonate, as a red brown solid melting at 528° C.

15 *1,1'-dimethyl-9,9'-o-phenylene-4,4'-quinazocarbocyanine-p-toluene sulphonate* having the structural formula



10

15

20

25 This salt was obtained from 4-methyl-mercapto-quinazoline, indene, and methyl-p-toluene sulphonate as green crystals melting at 298° C.

30 *1,1'-diethyl-9,9'-o-phenylene-4,4'-quinazocarbocyanine iodide* was prepared from 4-methyl-mercapto-quinazoline, indene, and ethyl-p-toluene sulphonate as green needles melting at 222° C.

35 *2,2'-dimethyl-3,4,3',4'-dibenz-7,7'-o-phenylene-thio-carbocyanine bromide* was prepared from 2-methylmercapto- $\beta$ -naphtha thiazole, methyl-p-toluene sulphonate and indene, as chocolate coloured needles with a gold reflux melting at 208° C.

40 The dye is a sensitiser for silver iodobromide emulsions and extends the sensitivity to about  $\lambda$  6300 Å. with a maximum at  $\lambda$  5800 Å.

45 *3,3'-dimethyl-2,2'-di-methylmercapto-o-phenylene-4,4'-pyrimido-carbocyanine-p-toluene sulphonates* having the structural formula



45

50

55 This salt was prepared from 2,4-di-methylmercapto-pyrimidine, indene and methyl-p-toluene sulphonate, as green rods melting at 306° C.

60 The dye is a sensitiser for silver iodobromide emulsions and extends the sensitivity to about  $\lambda$  6700 Å. with a maximum at about  $\lambda$  6100 Å.

65 *3,3'-diethyl-2,2'-di-methylmercapto-o-phenylene-4,4'-pyrimido-carbocyanine bromide* was prepared from 2,4-dimethylmercapto-pyrimidine, ethyl-p-toluene sulphonate, and indene, as green needles melting at 270° C.

70 The dye is a sensitiser for silver iodobromide emulsions and extends the sensitivity to about  $\lambda$  6600 Å. with a maximum at about  $\lambda$  5800 Å.

75 *1,1'-dimethyl-7,7'-o-phenylene-2,2'-pyridocarbocyanine iodide* was prepared from 2-methyl-mercaptopyridine, 3-methyl-p-toluene-sulphonate, and indene, as green prismatic needles melting at 268° C.

80 The dye is a sensitiser for silver chloride and iodobromide emulsions and sensitises over a band from about 4700 to 6400 Å. with a maximum at about 5500 Å.

75

3,3'-dimethyl-2,2',6,6'-tetramethylmercapto-o-phenylene-4,4'-pyrimido-carbocyanine-bromide having the structural formula



This salt was prepared from 2,4,6-trimethyl mercapto pyrimidine, indene, and methyl-p-toluenesulphonate, as a dark reddish green dyestuff.

The dye is a sensitiser for silver iodobromide emulsions and extends the sensitivity to about 6800 Å. with a maximum at about 6000 Å.

**I claim:**

- 1 chain:  
**20** 1. A 2,2'-dialkyl-7,7'-dimethenyl-thiocarbocyanine salt.  
 2. A 2,2'-dialkyl-7,7'-phenylene thiocarbocyanine salt.  
**25** 3. A 1,1'-dialphyl-9,9'-ethylene-2,2'-carbocyanine salt.

30 4. The process for the production of a new class of organic compounds comprising condensing in solution and in the presence of an acid binding agent, a compound selected from the group consisting of indene and cyclopentadiene with an alkyl quaternary salt of a heterocyclic nitrogen compound of the type used in the production of cyanine dyes, having a thioether group substituted in a position selected from the class consisting of  
35 alpha and gamma positions to the nitrogen atom.

alpha and gamma positions of the heterocyclic nitrogen compound. 5. The process of claim 4 wherein the alkyl quaternary salt of the heterocyclic nitrogen compound is formed in situ by reacting an alkyl salt with a compound selected from the group consisting of N-alkyl thione and alkyl mercapto bases of the corresponding heterocyclic nitrogen compound.

6. The process of claim 4 wherein the alkyl  
quaternary salt of the heterocyclic nitrogen com-  
45 pound is preformed by reacting an alkyl salt with  
a compound selected from the group consisting  
of N-alkyl thione and alkyl mercapto bases of  
the corresponding heterocyclic nitrogen com-  
pound.

7. A process for the production of a new class of organic compounds by condensing a compound selected from the group consisting of indene and cyclopentadiene with an alkyl quaternary salt of a heterocyclic nitrogen compound of the type used in the production of cyanine dyes having a thio-ether group substituted in a position selected from the class consisting of  $\alpha$  and  $\gamma$  positions to the nitrogen atom wherein said salt is prepared by fusing a compound selected from the group consisting of N-alkyl thiones and alkyl mercapto bases of the corresponding nitrogen compound with an alkyl salt in the presence of the compound selected from the class consisting of indene and cyclopentadiene, adding an acid binding solvent and heating to complete the condensation reaction.

8. The process of claim 4 wherein the alkyl quaternary salts of the heterocyclic nitrogen compounds containing thioether groupings are derived by reacting the corresponding heterocyclic nitrogen base containing a thione grouping with an alkyl salt. 20

9. The process of claim 4 wherein a compound selected from the group consisting of indene and cyclopentadiene is reacted with an alkyl quaternary salt of 1-methylmercapto-benzthiazole. 25

10. The process of claim 4 wherein a compound selected from the group consisting of indene and cyclopentadiene is reacted simultaneously with 1-ethyl-quinoline-2-thione and an alkyl salt. 30

11. A dye having the following general formula:



in which  $-\text{CR}_1=\text{CR}_2-$  is a grouping selected from the class consisting of  $-\text{CH}=\text{CH}-$  and



Y is an acid radical and X represents the atoms necessary to complete a heterocyclic radical of the type used in the production of cyanine dyes. 45

## JOHN DAVID KENDALL.

Certificate of Correction

Patent No. 2,153,927.

April 11, 1939.

JOHN DAVID KENDALL

It is hereby certified that errors appear in the printed specification of the above numbered patent requiring correction as follows: Page 1, first column, line 38, for "quaternary" read *quaternary*; page 2, second column, line 15, Example V, for "dimethenyl" read *dimethylene*; page 3, first column, line 38, Example XI, for "4'-dibenz-7,7-di-methyl-" read *4'-dibenz-7,7'-di-methenyl-*; page 5, second column, line 33, in the formula for "CR<sub>1</sub>=CR<sub>1</sub>" read *CR<sub>1</sub>=CR<sub>2</sub>*; and that the said Letters Patent should be read with these corrections therein that the same may conform to the record of the case in the Patent Office.

Signed and sealed this 1st day of August, A. D. 1939.

[SEAL]

HENRY VAN ARSDALE,  
*Acting Commissioner of Patents.*